

# UNITED STATES PATENT OFFICE.

JOHN MENSDORF, OF ETNA, PENNSYLVANIA.

## BATH FOR TREATING METALS.

SPECIFICATION forming part of Letters Patent No. 253,987, dated February 21, 1882.

Application filed December 22, 1881. (No specimens.)

*To all whom it may concern:*

Be it known that I, JOHN MENSDORF, of Etna borough, in the county of Allegheny and State of Pennsylvania, have invented a new 5 and useful Improvement in Baths for Treating Metals; and I do hereby declare the following to be a full, clear, and exact description thereof.

My invention relates to certain improvements in compositions or solutions for treating cast and malleable cast iron, its object being to "steelify" the cast or malleable iron, so as to render it hard, compact, and tough, so that it can be employed for many uses for 15 which the finer grades of steel have generally been employed.

To this end it consists in a bath for treating the metal composed of Jamestown weed, apples, turnips, and water in proper proportions, in which the casting, whether malleableized or not, is cooled after having been heated, so as to open its pores, this treatment toughening and hardening the metal and compacting the grain so as to impart to it the qualities of a fine grade of steel.

To enable others skilled in the art to use my invention, I will describe the same more fully.

My improved bath is composed of Jamestown weed, (*Stramonium*), one ounce, (1 oz.); apples, one ounce, (1 oz.); turnips, two ounces, (2 oz.); water, one gallon, (1 gal.) These ingredients are either scalded or boiled for a few minutes in part of the water and then 35 permitted to cool. The proportions of the ingredients may of course be somewhat varied; but I have found the proportions above set forth to work most satisfactorily when the remainder of the proportion of water is added, 40 though the entire proportion of water may be used in a boiling state at one time, and the bath then permitted to cool.

My improved bath may be employed to advantage both with the ordinary castings 45 formed from cast-iron and with the castings after having been decarburized by the ordinary methods of malleableizing cast-iron, the malleable iron being of course more tough and tenacious after treatment than the cast-

iron, but both being rendered more compact 50 in grain, hard or tempered, tough, and strong by my improved process. The castings are heated in a suitable furnace to a moderate heat, ordinarily known as a "cherry-red" heat, at which temperature the pores of the metal 55 are opened, so as to permit the bath or solution to penetrate entirely through the casting and produce the same effect throughout. A lower heat is not desirable, as it would not open the pores of the metal sufficiently, and 60 the desired result would not be obtained, or only the outer film would be affected, leaving the balance of the casting open in grain and liable to break. At a high heat the castings are liable to sag out of shape in the furnace and warp in cooling as well as to rapidly evaporate the water of the bath, so changing the proportions of the ingredients and impairing the effect of the bath. When brought to the proper heat, as aforesaid, the castings 70 are placed in the solution or bath previously made and allowed to cool therein, as is usual in tempering steel.

In order to regulate the degree of hardness to be imparted to the castings, instead of varying the solution, I generally employ urinia, this counteracting the other materials in proportion to the amount used, and increasing the toughness or tenacity of the metal. The amount used varies from one to three liquid 80 ounces, and by its use those skilled in the art can accurately regulate the temper of the article treated.

Articles treated in my improved bath, as above described, will be greatly improved in 85 quality, the treatment not only compacting the grain, but also imparting toughness, tenacity, and hardness to the casting. Where articles treated have been broken, the fracture shows that the grain has been compacted so 90 as to appear at least one-third closer than parts of the same casting before treatment, and to present much the same appearance as the grain of steel. Cast and malleableized articles so treated have been found as hard as 95 or harder than tempered steel and tougher, keeping their edge better and not being liable to chip off or break, so that articles so treated

are excellent for hammers, chasing, drilling, and planing tools, as well as for parts of machinery.

What I claim as my invention, and desire to secure by Letters Patent, is—

A bath for treating cast-iron or malleable cast-iron, composed of Jamestown weed, apples, turnips, and water, substantially in the proportions and for the purposes specified.

In testimony whereof I, the said JOHN MENSDORF, have hereunto set my hand.

JOHN MENSDORF.

Witnesses:

JAMES I. KAY,  
F. G. KAY.